

No. 830,040.

PATENTED SEPT. 4, 1906.

R. BAGGLEY, C. M. ALLEN & E. W. LINDQUIST.  
METHOD OF SMELTING ORES AND SEPARATING MATTES.

APPLICATION FILED FEB. 1, 1905. RENEWED JAN. 13, 1906.

6 SHEETS—SHEET 1.

Fig. 6.



II

Fig. 1.



II

WITNESSES:

Warren W. Gwartz  
H. M. Corwin

INVENTORS

Ralph Baggley  
Charles M. Allen  
Edward W. Lindquist  
by his attorney  
John A. Quinn  
his attorney

No. 830,040.

PATENTED SEPT. 4, 1906.

R. BAGGLEY, C. M. ALLEN & E. W. LINDQUIST.  
METHOD OF SMELTING ORES AND SEPARATING MATTES.

APPLICATION FILED FEB. 1, 1905. RENEWED JAN. 13, 1906.

3 SHEETS—SHEET 2

*WITNESSES:*

Warren W. Swartz  
St. M. Lorwin

INVENTORS

Kalte Gaffaley  
Charles H. Allen  
Edward W. Lindquist  
by Barker & Stevens  
Their atlys

No. 830,040.

PATENTED SEPT. 4, 1906.

R. BAGGLEY, C. M. ALLEN & E. W. LINDQUIST.  
METHOD OF SMELTING ORES AND SEPARATING MATTES.

APPLICATION FILED FEB. 1, 1905. RENEWED JAN. 13, 1906.

6 SHEETS—SHEET 3.

Fig. 3.



WITNESSES:

Warren W. Bartz  
H. M. Conine

INVENTORS

Ralph Baggley  
Charles M. Allen  
Edward W. Lindquist  
by Russell B. Rogers,  
their Atty.

No. 830,040.

PATENTED SEPT. 4, 1906.

R. BAGGALY, C. M. ALLEN & E. W. LINDQUIST.  
METHOD OF SMELTING ORES AND SEPARATING MATTES.

APPLICATION FILED FEB. 1, 1905. RENEWED JAN. 13, 1906.

6 SHEETS—SHEET 4.



Fig. 5.

Fig. 4.



WITNESSES:

Warren W. Swartz  
H. M. Cowen

INVENTORS:

Ralph Baggaley  
Charles M. Allen  
Edward W. Lindquist  
by Baskerville & Hayes  
their atty.

No. 830,040.

PATENTED SEPT. 4, 1906.

R. BAGGLEY, C. M. ALLEN & E. W. LINDQUIST.  
METHOD OF SMELTING ORES AND SEPARATING MATTES.

APPLICATION FILED FEB. 1, 1905. RENEWED JAN. 13, 1906.

6 SHEETS—SHEET 5.

Fig. 7.



WITNESSES

R. A. Balderson.  
Warren M. Gwartz

INVENTORS

Ralph Baggley,  
Charles M. Allen  
Edward W. Lindquist &  
John Allen, Jr.,  
Assignor to  
R. Baggley, C. M. Allen  
& E. W. Lindquist

No. 830,040.

PATENTED SEPT. 4, 1906.

R. BAGGLEY, C. M. ALLEN & E. W. LINDQUIST.

METHOD OF SMELTING ORES AND SEPARATING MATTES.

APPLICATION FILED FEB. 1, 1905. RENEWED JAN. 13, 1906.

6 SHEETS—SHEET 6

*Fig. 8.*



WITNESSES

*R. A. Balderson,  
Warren W. Swartz*

INVENTOR

*Ralph Baggley  
Charles M. Allen  
Edward W. Lindquist  
by his executors  
their atys*

# UNITED STATES PATENT OFFICE.

RALPH BAGGALEY, OF PITTSBURG, PENNSYLVANIA, CHARLES M. ALLEN, OF LO LO, MONTANA, AND EDWARD W. LINDQUIST, OF CHICAGO, ILLINOIS; SAID ALLEN AND LINDQUIST ASSIGNORS TO SAID BAGGALEY.

## METHOD OF SMELTING ORES AND SEPARATING MATTES.

No. 830,040.

Specification of Letters Patent.

Patented Sept. 4, 1906.

Application filed February 1, 1905. Renewed January 13, 1906. Serial No. 295,054.

*To all whom it may concern.*

Be it known that we, RALPH BAGGALEY, of Pittsburg, Allegheny county, Pennsylvania, CHARLES M. ALLEN, of Lo Lo, Missoula county, Montana, and EDWARD W. LINDQUIST, of Chicago, Cook county, Illinois, have invented a new and useful Method of Smelting Ores and Separating Mattes, of which the following is a full, clear, and exact description, reference being had to the accompanying drawings, forming part of this specification, in which—

Figure 1 represents a cross-section of a suitable converter in which to practice our invention, it being a cross-section on the line I I of Fig. 2. Fig. 2 represents a longitudinal cross-section on the line II II of Fig. 1, together with the blast-inlet pipe, hydraulic-power mechanism for tilting the vessel, the overflow-spout for the continuous discharge of slag and matte, the practically air-tight protecting cover for the slag and matte during their fall into the forehearth, and a portion of the forehearth itself. Fig. 3 represents one end elevation of the vessel with the hydraulic mechanism in section. Fig. 4 represents one side elevation of the vessel, in order to show the air-inlet, wind-box, and converting twyers, as well as the protected slag and matte overflow and a portion of the forehearth. Fig. 5 illustrates the rolling metal door, through which the overflow-spout may from time to time be examined and, if necessary, rodded by the operator. Fig. 6 represents in plan view the heavy bolted door or lid that covers the orifice, in the vessel, through which converter slags are delivered in the molten form for the purpose of extracting their contained mineral values. Fig. 7 represents the converter in end elevation and the hopper for the delivery of unfused ore thereinto. Fig. 8 is a transverse section of the converter, showing a refractory lining.

The objects of our invention may be briefly stated as follows: first, to utilize a primary bath in the new method of recovering values from ores by dissolving in a molten bath, described in United States Patent No. 766,654, issued August 2, 1904; second, to absorb and conserve the heat produced by the converting process; third, to operate continuously and practically without repairs to the apparatus; fourth, to provide a continuous method of

smelting that will utilize for fuel purposes the volatile portion contained in all sulfid ores; fifth, to provide a method of smelting that renders unnecessary the use of a blast-furnace with its heavy consumption of coke or other carbonaceous fuel and with its enormous percentages of loss of the volatile portion of ores under treatment, which losses are absolutely inseparable from blast-furnace practice of every kind; sixth, to provide a method of pyritic smelting that renders unnecessary the use of a hot blast that has been heated with carbonaceous fuel. To that end we preferably utilize apparatus such as that illustrated in the drawings, although apparatus of other construction—such, for instance, as water or air jacketed apparatus—may be utilized without departing from the spirit of our invention.

Referring now to the drawings, 2 in Fig. 1 represents the body of the converter, which in cross-section is preferably the segment of a circle, preferably about eighteen inches in thickness. We prefer to use blocks of copper, steel, wrought-iron, or cast-iron for this purpose; but other metals may be used.

3 illustrates the twyer-hole for the entrance of the converting-blast. It is preferably lined with seamless brass tubing 3' in order that when worn by the action of the punching-bars it may be readily and cheaply replaced. This converter is shown with bare metal walls; but it should be supplemented with a refractory lining 3", as illustrated in Fig. 8.

4 represents the removable top of the vessel, which is preferably made of heavy solid metal of sufficient thickness to successfully withstand the heat.

5 represents the reversible heavy metal ring with which the top of the vessel is provided. The holes 5' for the bolts or cap-screws that hold this ring in position are made to register accurately in order that the ring may be placed in many different positions in order to withstand the cutting effect of the molten metal or matte without renewal.

6 in Fig. 2 illustrates the charging door or inlet for ores.

In starting the process a bath of molten matte, preferably derived from the simple melting of sulfid ores, is provided from any

desired source. It may be melted within the vessel itself; but we prefer to provide the first bath with which the process is started from an outside source, because in this way we deliver into the vessel only a bath of matte free from silicious or aluminous slags and also one that is entirely free from the remnants of carbonaceous fuel, such as coke. Our experience has shown that coke is a very objectionable obstruction because it becomes enveloped in a non-conducting oxid coating of slag, and in this form it is infusible. After the first bath of matte has been charged into the vessel, which preferably is a bath derived, as above stated, from a simple melting of sulfid ores and as a consequence will contain heavy percentages of sulfur, iron, and other oxidizable elements and compounds, the converting-blast is turned on and heat is produced thereby within the interior of the vessel. This will be very great because we thus obtain most of the sulfur for fuel, whereas in a shaft-furnace about sixty-six per centum of it is lost through distillation and combustion. The escape of hot gases in this vessel will be choked, and for this reason the internal heat is retained to a great extent, thus materially aiding the process. Ore charges may be continuously or intermittently fed into the hopper 16. Such ore charges are preferably preheated by waste gases as a means of drying out the moisture contained in them and for the purpose of proportionately increasing the melting capacity of the vessel.

The converter, as illustrated in Fig. 2, is six feet in diameter and twenty feet long. It is provided with thirty-two blast twyers, each one and one-fourth inches in diameter. As the ore charges enter at the orifice 6 they drop onto a bath of hot matte on which they float and are dissolved during their travel toward the point of discharge. In marked contrast with this practice all past experiments in pyritic smelting have invariably been conducted in shaft-furnaces with ore columns and with certain percentages of carbonaceous fuel as the melting medium. Two things occur in connection with pyritic smelting in a shaft-furnace. First, the combustion of coke or other carbonaceous fuel is reducing in its action, and this is in conflict with the oxygen of the blast; second, the volatile portion of the sulfid ores is distilled, released, and escapes through the stack before the zone of actual fusion in the furnace is reached. In our present invention by submersion in a hot bath we catch and retain this volatile atom for use as fuel, and this has the effect of increasing by our present invention the fuel value of all sulfid ores treated by more than sixty-six per centum over that of all past experimenters.

It is intended that the entering blast shall be so great that at least a portion of its

oxygen will pass unconsumed through the molten bath and act as an oxidizing agent on the floating ore charge before the same has been dissolved. By this means we provide the equivalent of a hot blast without expense for carbonaceous fuel in preheating it. The ore-feed is purposely regulated so that the undissolved layer cannot sink to any great depth in the molten bath. Care is taken that the ore charges shall be fed into the vessel in such a manner and in such small amount at one time that an ore column cannot build up on the bottom of the vessel. In fact, the ore-feed is arranged so that the floating layer cannot at any time approach near to the level of the converting-twyers.

It is a well-known fact that slags are already oxidized compounds and that an air-blast delivered into any oxid is chilling in its effect. This is one reason that many attempts at pyritic smelting in shaft-furnaces have resulted in failure, because the chilling effect of the entering blast acting on the mingled ore, flux, and fuel, together with the enormous proportion of slag, soon solidifies the charge in the furnace.

From the point at which the ore charges enter the vessel, as shown at 6 in Fig. 2, they are compelled to travel a distance of preferably twenty feet, and during this travel they are subjected to the heat produced by a converting-blast while acting on a bath of matte that is purposely composed of ores—such, for instance, as sulfids, pyrrhotites, &c., that will furnish very high percentages of sulfur and iron and other oxidizable elements and compounds. We depend solely upon the heat thus produced to melt the entering ores, and in this way we eliminate the expense of coke or other carbonaceous fuel. In melting sulfid ores almost exclusively in this primary bath-producing vessel, and in producing the heat that results from this process our slags and mattes will always be very fluid. They flow out together in a continuous stream at 7 through one axis of the converter end the same as they flow at present through the overflow-spout of the ordinary blast-furnace. 8 illustrates a short overflow-spout which is preferably water-jacketed in order to successfully withstand the cutting action of the molten bath.

9 illustrates a practically air-tight cover and drop-tube which is intended to retain the original heat of the molten slag and matte during their passage from the primary converter into the forehearth. The joint at 10 is practically air-tight in order to prevent the entrance of air and at the same time to prevent any material escape of hot gases.

11 in Figs. 2 and 5 illustrates a rolling solid metal door, so arranged that it can be readily barred loose and rolled to one side should the slag or matte congeal upon it. Its object is to permit the operator to con-

stantly examine the discharge of slag and matte from the vessel through the overflow and, if necessary, to rod or to bar loose any chilled accretions that may form in this orifice.

12 represents the large forehearth.

13 represents the bottom of the forehearth.

14 represents a refractory bottom of the forehearth, which may be used or not, as preferred. The forehearth is preferably very large—say twenty feet in diameter, if circular, or, say, twenty feet long by eight or ten feet in width if a parallelogram. It is preferably made of heavy metal blocks, for the following reasons: First, that it shall conserve the original heats of the molten bath within it; second, that it shall be practically indestructible; third, that chilled accretions cannot build up on the bottom of it, and thus cause stoppages in the smelting operation, as is the case where a water-jacketed forehearth is used. Over the entire surface of the forehearth a coping or covering of congealed slag will form in this forehearth, the same as it does at present in all other forehearts. This congealed-slag-covering forms a practically air-tight junction with the solid metal drop-tube 9, so that the molten bath contained in the forehearth 12 itself, whether the same consist of slag or matte, or both, will be effectually thereafter protected against the chilling effects of the atmosphere. We have found in our work that this chilling effect is very great and that it is one of the numerous causes of undue losses of mineral values in the slag that is discharged to the dump.

In our present invention we retain the intense heat of both the matte and slag during their travel through a converter that is twenty feet in length. The molten bath of matte that exists continuously in the converter is so much greater than the comparatively small charge of ore that enters through the inlet 6 at one time that the ore is quickly congealed by the heat of the molten bath itself, and thus joins the bath without materially reducing its temperature. When the matte and slag pass beyond the heating influence of the converting-blast in the converter, and when they drop from the overflow-spout into the covered forehearth they are continuously protected against the chilling effects of the atmosphere, both in their fall and during their subsequent travel for a distance through the covered forehearth of approximately twenty feet. This affords ideal conditions for the separation of all mineral values contained in the slag, and it practically compels all matte prills to sink to the bottom of the forehearth and to join the body of molten matte, for which they naturally have a greater affinity than for the slag.

With the orifice 6 of the converter constantly closed by the ore in its hopper 16, while the blast is in operation and with the

converter-slag entrance closed during the progress of actual work, only two points of escape will remain for the hot gases that are constantly produced in large volume through the converting action. The one point of escape is through the nose of the converter into the stack and the second point of possible escape will be through the orifice 7. Through the latter they can only find their escape to the atmosphere after they have passed entirely under the congealed-slag covering of the forehearth and after they have reached the point of ultimate discharge of the worthless slag. Inasmuch as it is intended that the molten bath in the forehearth shall be in

actual contact with its congealed-slag covering, the escape of hot gases at this point will be unimportant. As before stated, these hot gases are produced in enormous volume and their exit from the converter is purposely choked in order to hold their heat within the vessel as a means of facilitating the process. This has the effect of creating considerable pressure within the converting vessel. Attention is called to the fact that the slags and mattes are thus maintained continuously at high temperatures until the point of ultimate discharge of the slag has been reached and also that these slags are exclusively discharged from the surface of a body of low-grade matte. Particular attention is called to the fact that converter-slags which may be high in mineral values are compelled to travel a distance of approximately forty feet under the most favorable possible conditions of heat and fluidity as a means of forcing a good separation. When ultimately discharged to the dump, they are thus discharged exclusively from the surface of a body of matte that is always low grade. These things taken together insure a better separation, cleaner slags, and much lower mineral losses than prevail in any present smelter-work.

Fig. 3 illustrates the method of delivering the blast to the wind-box 18. It also shows the rack 19 and pinion 20, whereby the converter is turned on its axis.

Fig. 4 illustrates the general proportions of the converting vessel, the blast-entrance, the hydraulic-power mechanism for revolving the converter, the overflow-spout, the covered drop-tube 9, and a portion of the forehearth 12.

Fig. 5 illustrates a detail of the drop-tube 9, as before explained.

22 in Figs. 1 and 6 designates a separate opening at the side of the opening 6, into which converter-slag derived from other converters in the series is poured in the molten state for the purpose of separating its contained mineral values.

Fig. 6 illustrates in plan view the orifice 22 and its heavy metal lid or door 21.

Fig. 7 illustrates the converter in end ele-

vation and showing the hopper and chute 16 for the delivery of the unfused ore into the converter that may be raised when the converter is rotated and that may be lowered for the feeding of ore charges.

This method of recovering mineral values from converter-slags is broadly new and as such we intend claiming it. It constitutes the most efficient method yet devised of accomplishing a close separation of mineral values contained in converter-slags, inasmuch as these converter-slags when poured into the opening 22 are compelled to travel the entire twenty feet through the converter 15 and thereafter the entire twenty feet through the forehearth and being discharged from the latter always over low-grade mattes will produce a cleaner slag than at present prevails, as hereinbefore described. The orifice 22 is provided with a heavy covering, so that it may be closed at all times as a means of preventing the escape of hot gases from the vessel, excepting when converter-slag is being poured into it. It will be noted that 25 under all ordinary circumstances this vessel while in actual operation will remain continuously in its upright position. It is only intended to be tipped or inverted like ordinary converters when it becomes necessary from 30 any cause to empty it.

Doubtless many modifications will suggest themselves to those skilled in the art without departing from the spirit of our invention, since

35 What we claim is—

1. The method of separating matte, which consists in supplying molten matte and ore to a converter, blowing air therethrough, and discharging the resultant matte and slag into 40 a forehearth or settling-chamber; substantially as described.

2. The method of separating matte, which consists in supplying molten matte and ore to a converter, blowing air therethrough, and 45 discharging the resultant matte and slag into a separate chamber and therein separating the matte from the slag; substantially as described.

3. The method of treating matte, which 50 consists in supplying molten matte to a converter, bessemerizing the matte, supplying ore thereto, melting the ore by the heat of the converting action, and discharging the resultant matte and slag into a separate chamber and therein separating the matte from the slag; substantially as described.

4. The method of smelting ore and separating matte, which consists in supplying a converter with a bath of molten matte, blowing air thereinto, feeding unfused ore into such bath in lesser volume relatively than the body of the molten matte, oxidizing and melting said ore, and delivering the resultant slag and matte into a separating vessel for

separation of the one from the other by gravity; substantially as described.

5. The method of smelting ore and separating matte, which consists in providing a converter with a molten bath of matte, feeding unfused ore charges into the converter at 70 or near one end, permitting such unfused ore to float in the direction of the opposite end of the converting vessel while subjected during its travel to the heat produced by the converting action and permitting the resultant 75 slag and matte to overflow into a separating vessel in which the matte may be separated from the slags by gravity; substantially as described.

6. The method of smelting ore and separating matte, which consists in providing a converter with a molten bath of matte, feeding unfused ore charges into the converter at or near one end of the vessel, permitting such unfused ore to float in the direction of the opposite end of the converting vessel while subjected during its travel to the heat produced by the converting action and permitting the resultant slag and matte to overflow continuously 80 at the axis of the converter into a separating vessel in which the matte may be separated from the slag by gravity; substantially as described.

7. The method of smelting ore and separating matte, which consists in providing a 95 converter with a molten bath of matte, feeding unfused charges of sulfid ore into the converter at or near one end of the vessel, permitting such unfused ore to float in the direction of the opposite end of the converting vessel while subjected during its travel to the heat produced by the converting action and permitting the resultant slag and matte to overflow continuously 100 at the axis of the converter into a separating vessel in which the matte may be separated from the slag by gravity; substantially as described.

8. The method of smelting ore and separating matte which consists in providing a 105 converter with a molten bath of matte, feeding such unfused ore charges into the converter at or near one end of the vessel, permitting such unfused ore to float in the direction of the opposite end of the converting vessel while subjected during its travel to the 110 heat produced by the converting action and permitting the resultant slag and matte to overflow continuously at the axis of the converter into a separating vessel in which the matte may be separated from the slag by gravity; substantially as described.

9. The method of smelting ore and separating matte which consists in providing a 115 converter with a molten bath of matte, feeding such unfused ore charges into the converter at or near one end of the vessel, permitting such unfused ore to float in the direction of the opposite end of the converting vessel while subjected during its travel to the 120 heat produced by the converting action and permitting the resultant slag and matte to overflow continuously at the axis of the converter and protecting them from the chilling action of the atmosphere during their travel from the interior of the converter into the interior of the forehearth, in which the matte may be separated from the slag by gravity; substantially as described.

9. The method of treating slag which consists in bessemerizing matte, moving the slag forwardly in contact with said matte to recover the mineral values, and discharging

the matte and slag into a forehearth or settling-chamber; substantially as described.

10. The method of treating converter-slag which consists in bessemerizing matte, moving the slag forwardly in contact with said matte to recover the mineral values, and discharging the matte and slag into a forehearth or settling-chamber; substantially as described.

In testimony whereof we have hereunto set to our hands.

RALPH BAGGAEY.  
CHARLES M. ALLEN.  
EDWARD W. LINDQUIST.

Witnesses:

AZELLE E. HOBART,  
WILLIAM M. KIRKPATRICK.